

# UNITED STATES PATENT OFFICE.

GEORG RICHTER, OF TEUTSCHENTHAL, NEAR HALLE-ON-THE-SAALE, GERMANY,  
ASSIGNOR, BY MESNE ASSIGNMENTS, TO THE CHEMICAL FOUNDATION, INC., A  
CORPORATION OF DELAWARE.

## PRODUCTION OF MOLYBDENUM COMPOUNDS.

1,360,581.

Specification of Letters Patent.

Patented Nov. 30, 1920.

No Drawing. Application filed July 12, 1917. Serial No. 180,196. Renewed April 19, 1920. Serial No. 375,151.

To all whom it may concern:

Be it known that I, Dr. GEORG RICHTER, a subject of the Empire of Germany, residing at Teutschenthal, near Halle-on-the-  
5 Saale, Germany, have invented new and useful Improvements Relating to the Production of Molybdenum Compounds, of which the following is a specification.

This invention relates to the process of  
10 treating ores or other material containing molybdenum, for instance wulfenite or slags containing molybdenum. For this purpose, the said materials for instance wulfenite after being sufficiently reduced to small  
15 pieces or to powder are treated with a watery solution of alkali sulfid, alkali polysulfid or alkali hydrosulfid, whereby molybdenum is dissolved in the form of alkali-sulfomolybdate, whereas lead is transformed  
20 to insoluble lead sulfid which remains in the residue. The extraction may be effected at ordinary or elevated temperature, and at ordinary or elevated pressure.

It is well known to produce alkali-sulfomolybdate solution and to precipitate from these molybdenum sulfid by adding an acid, but this method of operating is not desirable, as it requires very troublesome operations when carried out on a considerable  
25 scale. Applicant has found a suitable way for separating the sulfur from the alkali-sulfomolybdate and thus obtaining alkali-molybdate lyes sufficiently pure of producing molybdenum or molybdate compounds  
30 from them.

When the obtained sulfomolybdate lyes are treated with new quantities of wulfenite, oxygen is exchanged by sulfur and relatively pure solutions of alkali-molybdate are obtained, whereas lead sulfid is left in the  
35 residue:



Preferably both reactions—the extracting  
40 and the sulfur separating process—may be combined by effecting the extraction according to the counter-current principle, viz. by passing the alkali sulfid lye and the ore or other material in opposite directions  
45 through the extracting apparatus.

The sulfur may be separated from the

alkalisulfomolybdate lyes by other methods, for instance by treating them with other oxygenated lead compounds or with oxygenated iron, manganese or zinc compounds, 55 preferably with precipitated ferric hydroxid or protoxid of manganese.

In a modified form the process may be carried out in the following manner:—The ore or other material to be treated is reacted upon with a reduced quantity of alkali sulfid (or its equivalent) which is not sufficient to completely transform the molybdenum to alkalisulfomolybdate. In this case, the sulfomolybdate formed in the first place is then 60 at once transformed to alkali-molybdate, by the excess of unchanged wulfenite according to the above given equation.

The same end effect may be obtained by effecting the sulfurizing operation by a 65 smelting process. For this purpose, the ore or other material is melted with alkali sulfid in the well known manner, but only with a quantity of sulfid not sufficient to completely transform the molybdenum to alkali- 70 sulfomolybdate. On dissolving the molten mass, the reaction between the formed sulfomolybdate and the unchanged wulfenite takes place in the manner heretofore described.

In both cases it is not necessary to employ exactly the theoretical amount of alkali sulfid; an excess of sulfur can always be removed by fresh lead-ore or another desulfurizing agent. In the utmost case, this 75 method of separating the excess of sulfur may also be applied to solutions of alkali-sulfomolybdate which are produced by the known process of melting wulfenite with an excess of alkali sulfid and thereafter dissolving the molten mass.

When slags are to be treated I prefer to employ the melting process instead of the extracting process.

All reactions heretofore described may be 80 effected with ammonium sulfid or with mixtures generating ammonium sulfid instead of alkali sulfid.

Examples.—1. 100 kilograms of finely ground wulfenite are stirred during several 100 hours with a cold or hot watery solution of such a quantity of sodium sulfid as corre-

sponds to 25 kilograms of active sodium sulfid  $Na_2S$ . From the stirred mixture the solution practically containing all the molybdenum of the wulfenite in form of 5 sodium sulfomolybdate is separated from the formed lead sulfid by decanting and washing, and this solution is when cold stirred in another stirring apparatus with further 100 kilograms of finely ground wulfenite during one hour. From the stirred mixture a pure solution of sodium molybdate is obtained by filtering. The residue of wulfenite not yet completely changed to lead sulfid, which is left in the stirring apparatus, is stirred during some hours with the waste-water from the first operation and such an amount of sodium sulfid as corresponds to 20 kilograms of active sodium sulfid. After settling the solution of sodium sulfomolybdate which is standing above the lead sulfid is now separated from the sediment by decantation and transformed to sodium molybdate in another stirring apparatus by the addition of 100 kilograms of wulfenite, and so on.

2. 100 kilograms of finely ground wulfenite are melted with such a quantity of sodium sulfid as corresponds to 12 kilograms of active sodium sulfid, or the ore is stirred during several hours with a hot or cold watery solution of the sulfid.

The watery solution of the molten mass or the stirred mixture contains the molybdenum of the wulfenite in the form of sodium molybdate and may be separated from the lead sulfid formed along with it by filtering and washing.

It may be noted that where I have used the term "alkali sulfid" in the claims, this term is to include all kinds of compounds formed between sulfur and an alkali metal or the ammonium group represented for instance by the formulæ  $M_2S$ ,  $MHS$ ,  $M_2S_3$ ,  $M_2S_4$ ,  $M_2S_5$ , wherein  $M$  signifies sodium  $Na$  or potassium  $K$  or ammonium  $NH_4$ ; and where I have used the term "wulfenite" in the specification and claims, I mean the native lead molybdate.

I claim:

50 1. The herein described process of producing molybdenum compounds from material containing molybdenum consisting in extracting the said material with a watery

solution of alkali sulfid and treating the solution with a desulfurizing agent.

2. The herein described process of producing molybdenum compounds from material containing molybdenum, consisting in passing a stream of alkali sulfid lye and an excess of wulfenite in opposite directions, so that in the first instance a sulfomolybdate is formed which is then desulfurized by the excess of the wulfenite.

3. The herein described process of producing molybdenum compounds from material containing molybdenum, consisting in treating the said material with a sulfurizing agent and water and treating the solution thus obtained with a desulfurizing agent.

4. The herein described process of producing molybdenum compounds from material containing molybdenum, consisting in treating the said material with a sulfurizing agent and water and treating the solution thus obtained with wulfenite.

5. The herein described process of producing molybdenum compounds from material containing molybdenum, consisting in extracting an excess of the said ore with a watery solution of an alkali sulfid, the excess of the wulfenite acting as a desulfurizing agent on the alkali sulfomolybdate formed by the action of the alkali sulfid.

6. The herein described process of producing molybdenum compounds from material containing molybdenum, consisting in treating the said material with a mixture generating alkali sulfids when brought to reaction, and with water and treating the solution thus obtained with a desulfurizing agent.

7. The herein described process of producing molybdenum compounds from material containing molybdenum, consisting in treating the said material with a mixture generating alkali sulfids when brought to reaction and with water and treating the solution thus obtained with wulfenite.

In testimony whereof I affix my signature in presence of two witnesses.

DR. GEORG RICHTER.

Witnesses:

RUDOLPH FRICKS,  
THEKLA FRICKS.